

## 1

3,745,007

PROCESS FOR IMPROVING COLOR DEVELOPMENT  
ABILITY OF REVERSAL PHOTOGRAPHIC FILMS  
Tadashi Nagae, Nobuo Tsuji, and Takushi Miyazako,  
Kanagawa, Japan, assignors to Fuji Photo Film Co.,  
Ltd., Kanagawa, Japan  
No Drawing. Filed June 1, 1971, Ser. No. 148,903  
Claims priority, application Japan, June 1, 1970,  
45/47,035

Int. Cl. G03c 5/50, 1/72

U.S. Cl. 96—22

8 Claims

### ABSTRACT OF THE DISCLOSURE

There is provided an improvement in the conventional reversal color process, wherein a photographic element containing three photographic silver halide emulsion layers is subjected to (1) a first exposure to produce a latent image, (2) development in a photographic developer for producing a black-and-white negative image, (3) exposure to light of a color to which said first exposed silver halide emulsion layer is sensitive, and (4) a second development in a color developer for producing a colored image, said color developer containing an aromatic primary amine color developing agent and a photographic color coupler selected from the group consisting of a magenta forming pyrazolone color coupler, a cyan forming phenolic coupler, and a yellow forming open chain ketomethylene color coupler, the improvement comprising providing as a binder for said silver halide, gelatin and a specific water-soluble copolymer exhibiting a molecular weight of from 5,000 to 3,000,000 and further containing a specific repeating unit within its molecular structure.

### BACKGROUND OF THE INVENTION

#### (1) Field of the invention

The present invention concerns a color development of a coupler-free type reversal multilayer color photographic sensitive material and especially to a process for increasing an amount of dye produced in reversal color images.

#### (2) Description of the prior art

In the multilayer color photographic sensitive material containing a blue sensitive emulsion layer, a green sensitive emulsion layer and a red sensitive emulsion layer on a support, there are a coupler-containing type color sensitive material which contains silver halide and color formers (hereinafter it is called as "coupler") which form dyes by reacting with an oxidation product of an aromatic amine photographic developing agent in the photographic emulsion layers and a coupler-free type color sensitive material which does not contain couplers in the photographic emulsion layers (the coupler is included in the color developing solution). The present invention relates to such coupler-free type color sensitive material.

In the coupler-free color sensitive material, the following treatments are usually practiced in turn after exposing to light, that is, monochromatic white-black development, exposing to a red light at a support side of the sensitive material, cyan color development by a cyan color developer containing a cyan coupler and an aromatic amine photographic developing agent, exposing to a violet light at an emulsion side, yellow development by a yellow color developer containing a yellow coupler and an aromatic amine photographic developing agent, and magenta color development by a magenta color developer containing a magenta coupler and an aromatic amine photographic developing agent.

## 2

### SUMMARY OF THE INVENTION

#### Detailed description of the invention

The present invention concerns a new process for improving the density of reversal color images in the cyan color development, yellow color development and magenta color development, and especially to a new process for improving the density of magenta color images. According to the present invention, it is possible to obtain a more efficient color reproduction system and to produce a thinner emulsion layer by increasing the density obtained in the reversal color images. Accordingly, it is possible to improve sharpness and to economize silver halide in the emulsion layer.

The new process for improving the density of the reversal color images by the present invention comprises treating a silver halide gelatin emulsion containing the following water soluble polymer as the binder with color developer containing color couplers. The water soluble polymers used for the above-mentioned object, which have been found out by these inventors, are those having a repeated unit structure represented by the following formula:



wherein

$\text{R}_1$ : hydrogen atom or methyl group  
 $\text{R}_2$ : hydrogen atom or methyl group  
 $\text{R}_3$ : hydrogen atom or lower alkyl group (1-4 carbon atoms)  
 $X$  is a range of  $100 \geq x \geq 10$  which represents a ratio of both blocks represented by the above-mentioned rational formula. When  $x=100$ , it represents polyacrylamide.

Especially preferable polymers among these polymers are those having a number average molecular weight in a range of 5000-3,000,000. (Abbreviated as n.a.m.w.)

In the following, water soluble polymers used are shown, as exemplary, and not as limiting.

(1) Polyacrylamide (preferably 10,000-3,000,000 in n.a.m.w.)



(2) Acrylamide-acrylic acid copolymer (preferably 10,000-1,000,000 in n.a.m.w.)



(3) Acrylamide-methacrylic acid copolymer (preferably 10,000-1,000,000 in n.a.m.w.)



(4) Methacrylamide-acrylic acid copolymer (preferably 10,000-200,000 in n.a.m.w.)



(5) Methacrylamide-methacrylic copolymer (preferably 10,000-200,000 in n.a.m.w.)



(6) Methacrylamide-ethyl methacrylate copolymer (preferably 10,000-200,000 in n.a.m.w.)



As to the range of X is greater or equal 75 and smaller or equal 95 concerning from water soluble polymers 2 to 6.

The water soluble polymer used in the present invention may be added solely to a gelatin emulsion or may be added by substituting a part of gelatin in the emulsion. Though addition of the water soluble polymer may take place at any step before coating of the emulsion, it is preferable to add at the step from afterripening to coating. A preferable amount is in a range of 1%-90% particularly 5-50% (by weight) based on the combined amount (weight) of said gelatin and said copolymer.

According to this invention, good results are obtainable in the gelatin emulsion that contains silver bromoiodide as the silver halide. But it is possible to apply the present invention to many kinds of another silver halide-gelatin emulsions. The silver halide emulsion may be sensitized by compounds which contain labili sulfur such as sodium thiosulfate and allyl thiourea etc., and/or complex salts of monovalent gold and thiocyanic acid, and/or reduction sensitizers such as amino compounds and stannous chloride (refer to The Theory of the Photographic Process: 3rd edition; McMillan Company, New York (1966), pages 113-116), and/or polyalkylene oxide derivatives. In order to give green sensitivity and red sensitivity, the emulsion may include sensitizing dyes which sensitize a wavelength range of 500-700 m $\mu$ , for example, 1,1'-diethyl-2,2'-cyanine iodide and 3,3'-diethyl-9-methyl carbocyanine iodide (refer to the above-mentioned literature, pages 199-232). The emulsion may include stabilizers such as 4-hydroxy-6-methyl-1,3,3a,7-tetrazaindene (refer to the same literature, pages 344-346), hardeners such as formaldehyde and mucobromic acid (refer to the same literature, pages 54-60) and a wetting agents such as saponin and sodium alkylbenzene sulfonate.

Development of the multilayer color photographic material containing silver halide-gelatin emulsions which contain a water soluble polymer is carried out by a common reversal color processing for the coupler-free type sensitive material. Namely, at least a color developing agent and a diffusible coupler for cyan, magenta or yellow are included in each color developer. As the color developing agent, there are used well-known paraphenylenediamine derivatives such as 4-amino-N,N-diethyl-aniline, 4-amino-N,N-diethyl-3-methylaniline, 4-amino-3-methyl-N-methyl-N-( $\beta$ -methylsulfoanidoethyl)aniline and 4-amino-3-methyl-N-ethyl-N( $\beta$ -hydroxyethyl) aniline, etc. (refer to the above mentioned literature, page 387). As the diffusible cyan coupler, there are used well-known phenolic couplers such as 2-chloro-1-naphthol, 2,4-dichloro-1-naphthol, 2,4-dichloro-1-naphthol, 2(O-acetamido- $\beta$ -phenethyl)-1-hydroxy naphthamide, etc. (refer to the above-mentioned literature, page 387). As the diffusible magenta coupler, there are used open-chain methylene type couplers such as amylacetoneitrile, 2-cyanoethyl benzofuran and benzylacetoneitrile and cyclic methylene coupler such as 1-phenyl-3-(4-chlorobenzamido)-5-pyrazolone, 1-phenyl-3-(3-nitrobenzoylamino)-5-pyrazolone and 1-(2,4,6-trichlorophenyl)-3-(4-nitroanilino)-5-pyrazolone.

As the diffusible yellow coupler, there are used acylacetamide type open-chain methylene couplers such as 2-acetanilide, 2-aceto-2',4'-dichloroacetanilide, 2-benzoylacetanilide, 2-benzoyl-2'-methoxyacetanilide and 2-methyl-4-(methyl sulfonamidoethyl)ethylaniline, etc. (refer to the above-mentioned literature, page 389 and G. H. Brown et al., Journal of the American Chemical Society, 79 pages 2917-2927 (1957). These well-known color developing agents and couplers are used in combination.

A better understanding of the present invention will be

gathered from the following examples, which are merely illustrative and not limitative of the present invention.

#### EXAMPLE 1

5 After melting by heating a high-sensitive gelatino silver bromoiodide reversal color emulsion which was sulfur-sensitized and gold-sensitized (content of silver iodide: 3.5% by mol), it was wetted to a cellulose triacetate film base. Couplers were not included in the emulsion.

The binder of the silver bromoiodide in the coated emulsion was gelatin which contained polyacrylamide (molecular weight: 3,000,000, and molecular weight: 490,000) in many ratios. This emulsion layer was exposed to light by using a NSG II type sensitometer and processed to the following treatments.

|    |                                                                    | ° C. | Minutes |
|----|--------------------------------------------------------------------|------|---------|
| 1  | Prehardner bath                                                    | 27   | 1       |
| 2  | Water wash                                                         | 27   | 1       |
| 3  | Black and white                                                    | 27   | 4       |
| 4  | Water wash                                                         | 27   | 3       |
| 5  | Reversal exposure to white light                                   |      |         |
| 6  | Magenta development                                                | 27   | 5       |
| 7  | Water wash                                                         | 27   | 2       |
| 8  | Fix                                                                | 27   | 3       |
| 9  | Drying (sample taken for silver analysis)                          |      |         |
| 10 | Ferricyanide bleach                                                | 27   | 5       |
| 11 | Fix                                                                | 27   | 3       |
| 12 | Water wash and drying (sample taken for color density measurement) |      |         |

The various processing solutions has essentially the following compositions:

|    |                                                   |       |      |
|----|---------------------------------------------------|-------|------|
| 35 | Prehardener bath:                                 |       |      |
|    | Sulfuric acid (conc.)                             | cc    | 1.7  |
|    | Borax (10 hydrate)                                | g     | 20   |
|    | Potassium bromide                                 | g     | 2.3  |
| 40 | Sodium sulfate                                    | g     | 200  |
|    | 37% formaldehyde                                  | cc    | 10   |
|    | Sodium bisulfite                                  | g     | 1    |
|    | Water to make                                     | litre | 1    |
| 45 | Black and white developer:                        |       |      |
|    | N-methyl-p-aminophenol sulfate                    | g     | 5    |
|    | Anhydrous sodium sulfite                          | g     | 79   |
|    | Hydroquinone                                      | g     | 2    |
| 50 | Sodium carbonate (monohydrate)                    | g     | 40   |
|    | Potassium bromide                                 | g     | 3.5  |
|    | Potassium thiocyanate                             | g     | 20   |
|    | 0.1% potassium iodide                             | cc    | 12.5 |
| 55 | Sodium hydroxide                                  | g     | 1.0  |
|    | Water to make                                     | litre | 1    |
| 60 | Magenta developer:                                |       |      |
|    | Sodium sulfite                                    | g     | 5.0  |
|    | 4-amino-3-methyl-N,N-diethylaniline hydrochloride | g     | 2.0  |
| 65 | 1-phenyl-3-(3-nitrobenzoylamino)-5-pyrazolone     | g     | 1.4  |
|    | Sodium hydroxide                                  | g     | 2.5  |
|    | n-Butylamine                                      | cc    | 5    |
|    | Water to make                                     | litre | 1    |
| 70 | Ferricyanide bleach:                              |       |      |
|    | Ferricyanide                                      | g     | 60   |
|    | Potassium bromide                                 | g     | 20   |
|    | Water to make                                     | litre | 1    |
| 75 | Fix:                                              |       |      |
|    | Sodium thiosulfate                                | g     | 100  |
|    | Sodium sulfite                                    | g     | 15   |
|    | Water to make                                     | litre | 1    |

A ratio (by weight) of silver bromoiodide to the binder in the emulsion was 5 g. of binder (gelatin 100% by weight)/11 g. of silver bromoiodide. Data are shown in Table 1 in which gelatin of the binder is substituted by polyacrylamide in various ratios.

TABLE 1

| Ratio of polymer in binder of gelatin-polymer mixture (percent by weight) | Magenta D <sub>max.</sub> | Silver developed by color developer, mg. Ag/10 cm <sup>2</sup> | Magenta D <sub>max.</sub> /silver | 5  |
|---------------------------------------------------------------------------|---------------------------|----------------------------------------------------------------|-----------------------------------|----|
| 0% (polyacrylamide, molecular weight 3,000,000)                           | 1.9                       | 8.5                                                            | 0.23                              |    |
| 10% (polyacrylamide, molecular weight 3,000,000)                          | 2.1                       | 8.2                                                            | 0.26                              |    |
| 40% (polyacrylamide, molecular weight 3,000,000)                          | 2.3                       | 8.6                                                            | 0.27                              |    |
| 10% (polyacrylamide, molecular weight 490,000)                            | 2.3                       | 8.7                                                            | 0.26                              | 10 |
| 40% (polyacrylamide, molecular weight 490,000)                            | 2.4                       | 8.9                                                            | 0.27                              |    |

Increase of 15-20% or so of D<sub>max.</sub>/amount of silver was recognized when adding the polyacrylamide of the present invention as compared with no addition thereof. 15

## EXAMPLE 2

The same procedure was carried out as in Example 1 but using acrylamide-acrylic acid copolymer. 4 kinds of acrylamide-acrylic acid copolymer having approximately 100,000 of molecular weight in which x:(100-x)=90:10, 20 70:30, 50:50 and 30:70 and 4 kinds of said copolymer having approximately 2,000,000, 1,300,000, 700,000 and 100,000 of molecular weight in which x:(100-x)=70:30 25 were used.

Data are shown in Table 2.

TABLE 2

| Ratio of polymer in binder of gelatin-polymer mixture (percent by weight) | Magenta D <sub>max.</sub> | Silver developed by color developer, mg. Ag/10 cm <sup>2</sup> | Magenta D <sub>max.</sub> /silver | 30 |
|---------------------------------------------------------------------------|---------------------------|----------------------------------------------------------------|-----------------------------------|----|
| 0% M.W. 100,000 x:(100-x)=90:10                                           | 1.8                       | 8.3                                                            | 0.22                              |    |
| 10% M.W. 100,000 x:(100-x)=70:30                                          | 2.0                       | 8.0                                                            | 0.25                              | 35 |
| 10% M.W. 100,000 x:(100-x)=50:50                                          | 1.9                       | 7.0                                                            | 0.27                              |    |
| 10% M.W. 100,000 x:(100-x)=30:70                                          | 2.5                       | 8.7                                                            | 0.29                              |    |
| 10% M.W. 2,000,000 x:(100-x)=70:30                                        | 2.0                       | 8.0                                                            | 0.25                              |    |
| 10% N.W. 1,300,000 x:(100-x)=70:30                                        | 2.1                       | 7.9                                                            | 0.26                              |    |
| 10% M.W. 700,000 x:(100-x)=70:30                                          | 2.1                       | 8.2                                                            | 0.25                              | 40 |
| 10% M.W. 700,000 x:(100-x)=30:70                                          | 2.4                       | 8.5                                                            | 0.28                              |    |

Increase of 15-30% of D<sub>max.</sub>/amount of silver was recognized by adding the acrylamide-acrylic acid copolymers of the present invention.

## EXAMPLE 3

The same procedure as in the above-mentioned example was carried out but using acrylamide-methacrylic acid copolymer (M.W. approximately 100,000 x:(100-x)=50:50), methacrylamide-acrylic copolymer (M.W. approximately 100,000 x:(100-x)=30:70), methacrylamide-methacrylic acid copolymer (M.W. approximately 100,000 x:(100-x)=30:70) and acrylamide-ethyl methacrylate copolymer (M.W. approximately 100,000 x:(100-x)=70:30).

The resulting data are shown in Table 3.

TABLE 3

| Ratio of polymer in binder of gelatin-polymer mixture (percent by weight) | Magenta D <sub>max.</sub> | Silver developed by color developer, mg. Ag/10 cm <sup>2</sup> | Magenta D <sub>max.</sub> /silver | 65 |
|---------------------------------------------------------------------------|---------------------------|----------------------------------------------------------------|-----------------------------------|----|
| 0% acrylamide-methacrylic acid copolymer                                  | 2.2                       | 8.9                                                            | 0.25                              |    |
| 10% acrylamide-methacrylic acid copolymer                                 | 2.6                       | 9.0                                                            | 0.29                              |    |
| 10% methacrylamide-acrylic acid copolymer                                 | 2.8                       | 9.3                                                            | 0.30                              |    |
| 10% methacrylamide-methacrylic acid copolymer                             | 2.7                       | 8.7                                                            | 0.31                              |    |
| 10% acrylamide-ethyl methacrylate copolymer                               | 2.7                       | 9.5                                                            | 0.28                              | 70 |

Increase of 16-25% of D<sub>max.</sub>/amount of silver was recognized by addition of the copolymers of the present invention.

6  
EXAMPLE 4

Cyan color development was carried out (at 27° C. for 5 minutes) instead of the development by the magenta developing solution in the developing treatment of the emulsion layer in Example 2. Similarly, yellow color development was carried out (at 27° C. for 5 minutes) instead of the magenta development. The resulting data are shown in the following Table 4 and Table 5.

Formulations of the cyan color developer and the yellow color developer used are as follows.

## Cyan color developer:

|                                                    |       |     |
|----------------------------------------------------|-------|-----|
| Potassium bromide                                  | g     | 20  |
| 0.1% potassium iodide                              | cc    | 20  |
| Potassium thiocyanate                              | g     | 3.0 |
| Anhydrous sodium sulfite                           | g     | 10  |
| Sodium carbonate (monohydrate)                     | g     | 30  |
| Sodium hydroxide                                   | g     | 2.0 |
| 5-nitrobenzimidazolone nitrate                     | g     | 0.5 |
| 2,4-dichloro-1-naphthol                            | g     | 2.0 |
| 4-amino-3-methyl-N,N'-diethylaniline hydrochloride | g     | 3.0 |
| Water to make                                      | litre | 1   |

## Yellow color developing solution:

|                                                   |       |      |
|---------------------------------------------------|-------|------|
| Sodium sulfite                                    | g     | 5.0  |
| N,N'-diethyl-paraphenylenediamine                 | g     | 1.2  |
| Sodium carbonate (monohydrate)                    | g     | 20.0 |
| Potassium bromide                                 | g     | 0.3  |
| 0.1% potassium iodide                             | cc    | 20   |
| 2-benzoyl-(4'-paratoluenesulfonamide) acetanilide | g     | 1.0  |
| Sodium hydroxide                                  | g     | 4.0  |
| Water to make                                     | litre | 1    |

TABLE 4

| Ratio of polymer in binder of gelatin polymer mixture (percent by weight) | Cyan D <sub>max.</sub> | Silver developed by color developer, mg. Ag/10 cm <sup>2</sup> | Cyan D <sub>max.</sub> /silver |
|---------------------------------------------------------------------------|------------------------|----------------------------------------------------------------|--------------------------------|
| 0% polyacrylamide (M.W. 3,000,000)                                        | 1.2                    | 8.2                                                            | 0.15                           |
| 10% polyacrylamide (M.W. 3,000,000)                                       | 1.5                    | 9.0                                                            | 0.17                           |
| 10% polyacrylamide (M.W. 3,000,000)                                       | 1.5                    | 8.5                                                            | 0.18                           |

TABLE 5

| Ratio of polymer in binder of gelatin polymer mixture (percent by weight) | Yellow D <sub>max.</sub> | Silver developed by color developer, mg. Ag/10 cm <sup>2</sup> | Yellow D <sub>max.</sub> /silver |
|---------------------------------------------------------------------------|--------------------------|----------------------------------------------------------------|----------------------------------|
| 0% polyacrylamide (M.W. 3,000,000)                                        | 1.5                      | 8.9                                                            | 0.17                             |
| 10% polyacrylamide (M.W. 3,000,000)                                       | 1.8                      | 9.5                                                            | 0.19                             |
| 40% polyacrylamide (M.W. 3,000,000)                                       | 2.0                      | 10.0                                                           | 0.20                             |

Increase of D<sub>max.</sub>/amount of silver was recognized similarly at cyan development and yellow development.

What is claimed is:

1. In a photographic reversal color process, wherein a photographic element containing three photographic silver halide emulsion layers is subjected to:

- (1) a first exposure to produce a latent image therein,
- (2) development in a photographic developer for producing a black-and-white negative image,
- (3) exposure to light of a color to which said first exposed silver halide emulsion layer is sensitive, and
- (4) a second development in a color developer for producing a colored image,

said color developer containing an aromatic primary amine color developing agent and a photographic color coupler selected from the group consisting of a magenta forming pyrazolone color coupler, a cyan forming phenolic coupler, and a yellow forming open chain ketomethylene color coupler, the improvement which comprises:

providing a binder for said silver halide consisting essentially of a gelatin and a water-soluble copolymer exhibiting a molecular weight ranging from 5,000 to 3,000,000, characterized as containing as a repeating unit within said copolymer, a structure of the following formula:



wherein  $\text{R}_1$  represents a member selected from the group consisting of a hydrogen atom and a methyl group;  $\text{R}_2$  represents a member selected from the group consisting of a hydrogen atom and a methyl group;  $\text{R}_3$  represents a member selected from the group consisting of a hydrogen atom and a lower ( $\text{C}_1$ - $\text{C}_4$ ) alkyl group; and  $x$  represents a range of

$$100 \geq x \geq 10$$

2. The process of claim 1, wherein said copolymer is an acrylamide-acrylic acid copolymer.
3. The process of claim 1, wherein said copolymer is an acrylamide-methacrylic acid copolymer.

4. The process of claim 1, wherein said copolymer is a methacrylamide-acrylic acid copolymer.

5. The process of claim 1, wherein said copolymer is a methacrylamide-methacrylic acid copolymer.

6. The process of claim 1, wherein said copolymer is a methacrylamide-ethyl methacrylate copolymer.

7. The process of claim 1, wherein said copolymer is present in an amount ranging from 1 to 90% by weight, based on the combined weight amount of said gelatin and said copolymer.

8. The process of claim 1, wherein said copolymer is present in an amount ranging from 5 to 50% by weight, based on the combined weight amount of said gelatin and said copolymer.

15

#### References Cited

##### UNITED STATES PATENTS

3,592,215 8/1971 Abel, et al. ----- 96—114

20 RONALD H. SMITH, Primary Examiner

A. T. SURO PICO, Assistant Examiner

U.S. Cl. X.R.

96—114